

United States Patent [19]  
Kawai et al.

[11] 3,940,271  
[45] Feb. 24, 1976

[54] COLOR PHOTOGRAPHIC  
LIGHT-SENSITIVE MATERIAL

[75] Inventors: **Masayoshi Kawai; Tadao Shishido; Shoji Ishiguro; Tadao Sakai**, all of Kanagawa, Japan

[73] Assignee: **Fuji Photo Film Co., Ltd.**, Minami-ashigara, Japan

[22] Filed: **Feb. 4, 1974**

[21] Appl. No.: **439,675**

[30] Foreign Application Priority Data

Feb. 2, 1973 Japan ..... 48-13514

[52] U.S. Cl. .... 96/4; 96/55; 96/60 R; 96/60 BF; 96/74

[51] Int. Cl. <sup>2</sup> .. G03C 7/24; G03C 7/00; G03C 5/32; G03C 1/76

[58] Field of Search ..... 96/66.3, 64, 4, 74, 39, 96/60 R, 55

[56] References Cited

UNITED STATES PATENTS

3,046,130 7/1962 Dersch et al..... 96/66.3

|           |         |                    |         |
|-----------|---------|--------------------|---------|
| 3,084,044 | 4/1963  | Dersch et al.....  | 96/66.3 |
| 3,705,799 | 12/1972 | Bello et al.....   | 96/4    |
| 3,723,125 | 3/1973  | Hayashi et al..... | 96/74 X |

Primary Examiner—Charles L. Bowers, Jr.

Assistant Examiner—Alfonso T. Suro Pico

Attorney, Agent, or Firm—Sughrue, Rothwell, Mion, Zinn & Macpeak

[57]

ABSTRACT

A color photographic light-sensitive material comprising a support having coated thereon at least one light-sensitive silver halide emulsion layer containing a yellow dye-forming coupler, at least one light-sensitive silver halide emulsion layer containing a magenta dye-forming coupler, at least one light-sensitive silver halide emulsion layer containing a cyan dye-forming coupler, and at least one light-sensitive silver halide emulsion layer containing a compound having a thioether bond directly connected to a nitrogen-containing heterocyclic ring.

13 Claims, No Drawings

## COLOR PHOTOGRAPHIC LIGHT-SENSITIVE MATERIAL

### BACKGROUND OF THE INVENTION

#### 1. FIELD OF THE INVENTION

The present invention relates to a color photographic light-sensitive material, and more particularly it relates to a color photographic light-sensitive material capable of recording sound images.

#### 2. DESCRIPTION OF THE PRIOR ART

As recording methods for sound images for color photographic light-sensitive materials, an optical recording system and a magnetic recording system are generally known. The present invention relates to the photographic materials suitable for the optical recording system.

Color print films, color reversal films, color reversal print films, etc. are used as the color photographic light-sensitive materials for movies and for television. Sound images are optically recorded with color images on the color photographic light-sensitive materials, and are reproduced by converting the sound signals recorded as the optical density or areas in the materials into light-signals, then converting the light-signals into electric signals using a light-receiving device, and further converting the electric signals into sound signals. In the reproduction steps of sound images, phototubes having various optical characteristics have been used as the light-receiving device. The most typical phototube which is called an "S-1 type" has an optical absorption maximum at about  $800\mu$  in the infra-red region (for example, as disclosed in Adrin Cornwell, *Color Cinematography*, page 593 (1951)).

On the contrary, color dyes, which are formed by the coupling reaction of color couplers and the oxidation products of color developing agents, such as the p-phenylenediamines, according to the subtractive color photography, all have a main absorption within the visible region, and therefore the main absorption of the dyes does not correspond to the optical characteristics of the above-described phototube. Accordingly, sound reproductions based on only color dye images are weak and impractical. For the purpose of more practical sound reproductions of color photographic light-sensitive materials, silver images or silver sulfide images are formed on the sound track areas of the color photographic light-sensitive materials in the developing process, and the optical density in the infra-red region of the images is utilized for sound reproductions. In this case, the optical density in the infra-red region (transmitting density) is usually about 1.0 to 1.6.

The sound track areas of color print films can be produced using the processing steps disclosed in the *Journal of the Society of Motion Picture and Television Engineers*, Vol. 77, page 1154 (1968). According to this method, color images of image portions and sound images of sound track areas are simultaneously developed in a color developing bath. In a first fixing bath, the unexposed silver halide is removed and in a bleaching bath, the developed silver formed in the developing step is rehalogenated. In a sound developing step, the silver halide corresponding to only the sound track areas is converted into silver images by coating a viscous sound developer on the sound track areas, selectively. In a second fixing bath, the silver halide in the image portions is removed, and in a stabilizing bath, the dye image are stabilized. Thus, the optical density in

the infra-red region of the silver images on the sound track areas can be utilized for sound reproductions.

As described above, it is necessary in the production of the sound track areas of color films to form silver or silver sulfide images using processing steps other than the color image forming steps. The reason why the sound track areas containing silver or silver sulfide images is needed is due to the optical characteristics of the phototube used for the sound reproductions which requires an absorption maximum in the infra-red region and that the color dyes formed by color development do not have sufficient optical density in this region.

Color photographic light-sensitive materials capable of forming sound track areas which do not require the special processing steps as described above have been proposed (U.S. Pat. Nos. 3,705,801; 3,715,208; and 3,737,312; and U.S. patent application Ser. No. 360,507, filed May 15, 1973). The color photographic light-sensitive materials include an auxiliary layer capable of forming silver images upon color development and which are not bleached in a bleaching step. In the auxiliary layer, developable silver is hardly formed by imagewise exposure, but only in the sound track areas of the layer, silver for sound images is formed which is not bleached in the following bleaching step and hence remains in the layer. Therefore, photographic materials including the auxiliary layer have the advantage that the selective coating of a viscous sound developer on the sound track areas can be omitted. Further, with these photographic materials, since the silver images formed in the sound track areas by color development can be used as the sound images, the rehalogenation step of the developed silver is unnecessary, and the bleaching and fixing step can be carried out in the same bath, whereby the processing steps are simplified.

A color photographic light-sensitive material is composed of a support having coated thereon silver halide emulsion layers having different optical sensitivities. The photographic material is developed, after imagewise exposure, with a color developer, whereby color dye images and silver images are formed. Then, the material is bleached in a bleaching step, whereby the silver images are oxidized, and is fixed in a fixing step, whereby the silver halide is removed and a color photograph containing the color dye images can be obtained.

The above described color photographic light-sensitive material has a layer capable of forming silver images which are not removed by the bleaching and fixing steps, and gives, by conventional color development, a color photograph containing color dye images and silver images that are advantageously utilized as sound track areas.

As an advantageous method for forming the silver images which are not removed by the processing steps, the following compounds are proposed. That is, when the compound is incorporated into a silver halide emulsion layer, it remarkably reduces the rate at which silver is removed in the bleaching and fixing steps or it causes the silver to lose its ability to be removed in these steps. The compound can have the property in which the silver is removed in some degree only in the initial period of these steps but that the silver is not substantially removed after the initial period. Such a compound is defined as a bleach inhibitor in the specification.

As bleach inhibitors, a compound having a mercapto group is disclosed in Japanese Patent Application laid open to public inspection No. 13482/72. However,

since a bleach inhibitor is also considered to be a development inhibitor or a chemical inhibitor, it is difficult to obtain a higher optical density of silver even if it is used. Namely, where a large amount of the bleach inhibitor is used, the amount of silver remaining after the bleaching step is small because the amount of the developed silver is small due to the development inhibitor while the bleach inhibiting effect is higher. On the other hand, where a small amount of the bleach inhibitor is used, the amount of silver remaining after the bleaching step is also small because the bleach inhibiting effect is lower while the amount of the developed silver is greater due to less development inhibition.

An object of the invention is, therefore, to provide a bleach inhibitor capable of providing sufficient optical density in the infra-red region without or with little development or chemical inhibition.

Another object of the invention is to provide a color photographic light-sensitive material capable of providing sufficient optical density in the infra-red region which does not require special processing steps as in the conventional method to produce sound track areas by using a novel bleach inhibitor.

Still another object of the invention is to provide a method for forming sound images having higher sound quality which does not involve special processing steps as in the conventional method.

#### SUMMARY OF THE INVENTION

The above objects of the invention can be attained by using as a bleach inhibitor a compound having a thioether directly connected to a nitrogen-containing heterocyclic ring. That is, according to the present invention, a color photographic light-sensitive material can be provided comprising a support having coated thereon at least one light-sensitive silver halide emulsion layer containing a yellow color-forming coupler, at least one light-sensitive silver halide emulsion layer containing a magenta color-forming coupler, at least one light-sensitive silver halide emulsion layer containing a cyan color-forming coupler and at least one light-sensitive silver halide emulsion layer containing a compound having a thioether directly connected to a nitrogen-containing heterocyclic ring.

#### DETAILED DESCRIPTION OF THE INVENTION

According to one embodiment of the invention, a light-sensitive material comprises a support having coated thereon a first silver halide emulsion layer containing a coupler forming a yellow dye when reacted with the oxidation product of a color developing agent and having a light-sensitivity in a first region of visible light, a second silver halide emulsion layer containing a coupler forming a magenta dye when reacted with the oxidation product of a color developing agent and having a light-sensitivity in a second region of visible light, a third silver halide emulsion layer containing a coupler forming a cyan dye when reacted with the oxidation product of a color developing agent and having a light-sensitivity in a third region of visible light, and a fourth silver halide emulsion layer containing a bleach inhibitor and having a light-sensitivity in the ultra violet region, visible region or infra-red region.

When the color photographic light-sensitive material is imagewise exposed through an original, and then developed with a color developer, yellow dye images and silver images are formed in the first silver halide emulsion layer, magenta dye images and silver images

are formed in the second silver halide emulsion layer, cyan dye images and silver images are formed in the third silver halide emulsion layer, and silver images are formed in the fourth silver halide emulsion layer. Then, the color photographic material is bleached, whereby the silver images in the first, second and third silver halide emulsion layers are bleached but the silver images in the fourth silver halide emulsion layer are not bleached due to the action of the bleach inhibitor and remain. Thus, a color photograph having color dye images and silver sound images is obtained.

The fourth silver halide emulsion layer can have a light-sensitivity to the ultra violet region, the visible region or the infra-red region. However, this silver halide emulsion layer must not form developable silver which gives an optical density in such a degree that the silver adversely influences the color reproduction under usual imagewise exposure. Accordingly, if the light-sensitive region of the fourth silver halide emulsion layer overlaps those of the first, second and third silver halide emulsion layers, it is desirable that the sensitivity of the fourth silver halide emulsion layer be  $\frac{1}{4}$  or less, preferably  $1/6$  or less, the sensitivities of the other layers.

Alternatively, the sensitivity region of the fourth silver halide emulsion layer can be provided between the sensitivity regions of the first and second silver halide emulsion layers and/or between the sensitivities of the second and third silver halide emulsion layers. These methods, i.e., this method and that described above, can be used in combination. By applying these methods the formation of a silver image in the fourth silver halide emulsion layer in an amount undesirable for color photographic images can be prevented.

In the light-sensitive material of the invention, a silver halide emulsion layer containing a bleach inhibitor is further coated in addition to a blue-sensitive emulsion layer, a green-sensitive emulsion layer and a red-sensitive emulsion layer of the conventional color photographic light-sensitive material.

As a preferred embodiment of the invention, the photographic material comprises a support having coated thereon, in order from the support, a blue-sensitive silver halide emulsion layer containing a yellow dye-forming coupler, a red-sensitive silver halide emulsion layer containing a cyan dye-forming coupler, a green-sensitive silver halide emulsion layer containing a magenta dye-forming coupler and a green-sensitive silver halide emulsion layer containing a bleach inhibitor.

In this case, two green-sensitive silver halide emulsion layers, i.e., the green-sensitive layer containing the magenta dye-forming coupler and the green-sensitive layer containing the bleach inhibitor, can be coated in the reverse order. In all cases, the emulsion layer containing the bleach inhibitor can have an optical sensitivity in the ultra violet region, the visible region or the infra-red region.

As another preferred embodiment of the invention, the silver halide emulsion layers containing the dye-forming couplers can be coated on a support in an order different from the above embodiment, for example, in the order on a support of a blue-sensitive layer containing a yellow dye-forming coupler, a green-sensitive layer containing a bleach inhibitor, a red-sensitive layer containing a cyan dye-forming coupler and a green-sensitive layer containing a magenta dye-forming coupler or in the order on a support of a green-sensitive

layer containing a bleach inhibitor, a blue-sensitive layer containing a yellow dye-forming coupler, a red-sensitive layer containing a cyan dye-forming coupler and a green-sensitive layer containing a magenta dye-forming coupler.

A bleach inhibitor represented by the following general formula (I) is quite advantageous in this invention and is preferred,

groups. Suitable substituents which can be present are alkoxy groups such as methoxy, ethoxy, etc., hydroxy, sulfo, carboxy, amino, etc.

An alkylimidazole compound represented by the general formula (I) can be in the free form or in a salt form. The salt can be formed using usual salt-forming agents such as hydrogen halides, perchloric acid, sulfuric acid, nitric acid, etc.

The following compounds are typical examples of compounds of the general formula (I).



wherein R is an alkyl group having not less than 12 carbon atoms, with the alkyl group being both substituted or unsubstituted. Generally, an alkyl group having up to 20 carbon atoms can suitably be used. Suitable examples of such alkyl groups are dodecyl, tetradecyl, pentadecyl, hexadecyl, oleyl, octadecyl, etc.

These compounds can be easily synthesized by the reaction of ethylene thiourea and an alkyl halide as described in *Analytical Chemistry*, vol. 32, page 55 (1966).

Since the compound represented by the general formula (I) is non-diffusible, *per se*, and does not diffuse into color image-forming layers, silver images do not remain in the color image-forming layers.

The bleach inhibitor having thioether bond of the invention is different from the mercapto compound described in U.S. Pat. No. 3,715,208 in its chemical structure and its properties. That is, while the mercapto

compound forms a mercapto silver salt in the presence of silver ion, the bleach inhibitor of the invention does not form mercapto silver salt under the same conditions. This is proved from the results of argentometric (potential) titration which is carried out using the bleach inhibitors (1) and (3) of the invention, and the compound (A) having a mercapto group.

Compound (A)  $\text{HS}-\text{C}_{12}\text{H}_{25}$

The silver potential is measured by dissolving  $1 \times 10^{-3}$  mol of each compound in methanol, adding a buffer to each solution to adjust the pH to 5.0, 7.0, 9.0 and 11.0, and then adding dropwise an aqueous silver nitrate solution at the rate of one equivalent per 5 minutes at 50°C. The buffer each is an acetate buffer for the pH of 5.0, a maleate buffer for the pH of 7.0, and a borate buffer for the pH of 9.0 and pH 11.0. The results obtained are shown in the following table.

inhibiting action is obtained. Thus, a higher optical density in the infra-red region and higher a sound quality can be obtained.

The amount of the bleach inhibitor which can be added to the light-sensitive material of this invention, although it will differ depending on the characteristics of the inhibitor and emulsions used, is usually about  $1 \times 10^{-7}$  to  $1 \times 10^5$  g, preferably about  $1 \times 10^{-5}$  to  $1 \times 10^4$  g, per 1 mol of silver in the emulsion layer to which it is added.

Examples of the preferable supports on which the lightsensitive silver halide emulsion layers are coated are a cellulose ester film such as a cellulose nitrate film or a cellulose acetate film; a polyester film such as a polyethylene terephthalate film; a polyvinyl chloride film; a polystyrene film; a polycarbonate film, etc.

The hydrophilic colloid which can be used in the

| pH   | Buffer Only<br>(Volts) | Bleach Inhibitor (1)    |                         | Bleach Inhibitor (3)    |                         | Compound (A)<br>(Volts) |
|------|------------------------|-------------------------|-------------------------|-------------------------|-------------------------|-------------------------|
|      |                        | 1 Equivalent<br>(Volts) | 2 Equivalent<br>(Volts) | 1 Equivalent<br>(Volts) | 2 Equivalent<br>(Volts) |                         |
|      |                        |                         |                         |                         |                         |                         |
| 5.0  | + 0.54                 | + 0.28                  | + 0.55                  | + 0.54                  | + 0.04                  | + 0.55                  |
| 7.0  | + 0.52                 | "                       | + 0.51                  | + 0.52                  | - 0.04                  | + 0.52                  |
| 9.0  | + 0.53                 | "                       | + 0.52                  | + 0.53                  | - 0.08                  | + 0.51                  |
| 11.0 | + 0.40                 | "                       | + 0.41                  | + 0.39                  | - 0.13                  | + 0.41                  |

In the table, since silver potential (+ 0.28 volt) of the bleach inhibitor (1) to one equivalent of silver has no relation to the pH value and the silver potential of the bleach inhibitor (3) to two equivalents of silver is not shown, it is believed that these silver potentials depend on the silver potential of silver bromide. Also, it is believed that all silver potentials of the bleach inhibitor (1) to two equivalents of silver, the bleach inhibitor (3) to one equivalent of silver and the compound (A) to two equivalents of silver depend on the silver potential of the buffer. Further, it is believed that the silver potential of + 0.04 volt, - 0.04 volt, - 0.08 volt and - 0.13 volt at pH 5.0, pH 7.0, pH 9.0 and pH 11.0 of the compound (A) each depends on the silver potential of the mercapto silver. From the results that the bleach inhibitors (1) and (3) do not show reducing values, it is apparent that they can not form mercapto silver at a pH of 5.0 to 11.0.

The bleach inhibitor of the invention does not have a mercapto group in the structure and does not produce the mercapto group during the preparation of the photographic material and during the photographic processes thereof.

The bleach inhibitor of the invention has the following advantage in comparison with a compound having a mercapto group. That is, the mercapto compound is strongly adsorbed on the silver particles, whereby the bleaching of silver is reduced. However, since the mercapto compound is adsorbed on silver halide particles, similarly, the optical density of the developed silver, as a result thereof, is reduced. It is, therefore, impossible to obtain a sufficient optical density in the infra-red region and to obtain higher sound quality. On the contrary, the bleach inhibitor of the invention is not adsorbed on silver halide particles but is selectively adsorbed on only silver particles, whereby the silver particles are protected from bleaching. Accordingly, the optical density of the silver is not reduced as in the case of using a mercapto compound and a stronger bleach

silver halide emulsion layer includes all of those known in the art. Advantageously gelatin, acylated gelatin such as described in U.S. Pat. No. 2,614,928, grafted gelatin such as described in U.S. Pat. Nos. 2,831,767; 2,763,625; and 2,956,884, albumin, gum arabic, agar, a cellulose derivative (e.g., an alkyl ester of carboxy cellulose, hydroxyethyl cellulose, carboxymethyl hydroxyethyl cellulose), and a synthetic resin (e.g., polyvinyl alcohol, polyvinyl pyrrolidone) can be used. These hydrophilic colloids also can be preferably used as a binder for a photographic layer other than the emulsion layer, such as a protective or uppermost layer, a filter layer, an intermediate layer, an antihalation layer, a subbing layer or a backing layer.

The hydrophilic colloid used for the photographic layers of the light-sensitive material can be advantageously hardened using hardeners such as aldehydes, methylols, 1,4-dioxanes, azirazines, isooxazoles, carbodiimides, active halogen compounds or active vinyl compounds, for example, as described in U.S. Pat. Nos. 3,232,764; 3,288,775; 2,732,303; 3,635,718; 3,232,763; 2,732,316; 2,586,168; 3,103,437; 3,017,280; 2,983,611; 2,725,294; 2,725,295; 3,100,704; 2,091,537; 3,321,313, etc.

In the light-sensitive materials of the invention, all silver halide emulsions known in the photographic art can be used. As such silver halides, there are silver bromide, silver iodobromide, silver chlorobromide, silver chloroiodobromide, silver chloride, etc. A so-called converted type silver halide particles disclosed in U.S. Pat. Nos. 2,592,250 and 3,622,318 and British Pat. No. 635,841 can also be advantageously used.

The silver halide emulsion can be chemically sensitized using active gelatin or with a sulfur compound. It can be also chemically sensitized with a noble metal salt such as palladium or gold, a reducing agent such as a stannous salt or a polyalkylene derivative as described in U.S. Pat. Nos. 1,574,944; 1,623,499; 2,410,689; 2,448,060; 2,399,083; 2,642,361; and

2,487,850. The emulsion can be further spectrally sensitized with a cyanine or merocyanine dye as described in U.S. Pat. Nos. 2,519,001; 2,666,761; 2,734,900; 2,739,964; and 3,481,742. The emulsion can contain a stabilizer such as a mercury compound or an azaindene, a plasticizer such as glycerol as described in C. E. K. Mees and T. H. James, *The Theory of the Photographic Process*, pages 53 - 54, The Macmillan Co., New York (1966) and in U.S. Pat. Nos. 2,904,434; 2,940,854, etc., or a coating aid such as saponin or polyethylene glycol monolaurylether as described in U.S. Pat. Nos. 3,663,229; 3,619,199; 3,617,292; 3,545,974; 3,607,291; 3,589,906; 3,539,152; 3,564,576; 3,514,253; 3,666,478; 3,506,449; 3,514,293; and 3,493,379. Further, it can contain an antistatic agent as described in U.S. Pat. No. 2,739,888, an ultraviolet absorbent as described in U.S. Pat. Nos. 2,415,624; 3,052,636; 3,074,971; 3,085,097; 3,069,456; 3,215,536; 2,719,086; 2,537,877; 2,739,888; 2,784,087; 2,882,150; 2,875,053; 2,739,971; 3,097,100; 3,060,029; 2,632,701; 2,888,346; and 2,748,021, an optical brightening agent as described in U.S. Pat. Nos. 3,630,738; 3,615,544; 3,586,673 and 3,434,837 and British Pat. Nos. 1,332,475; 1,319,763; and 1,333,586, etc.

In the present invention, all kinds of open-chain keto-methylene type yellow dye-forming couplers can be advantageously used. Typical examples of these couplers include benzoyl acetoanilide type couplers and pivaloyl acetoanilide type couplers. All kinds of magenta dye-forming couplers such as pyrazolones or indazolones also can be advantageously used. Further, all kinds of cyan dye-forming couplers such as the phenols or naphthols can be advantageously used. These couplers can have a coupling-off group connected to the active carbon atoms at the coupling position. In these couplers, it is preferable that they have a ballast group in the molecule, whereby they are rendered non-diffusible. The terms "coupling-off group", "ballast group" and "non-diffusible" are used as they are generally used in the art with respect to color couplers, and can be easily understood by one skilled in the art. More preferable color couplers in the invention are selected from the group consisting of yellow dye-forming couplers which react with the oxidation product of a color developing agent to form yellow dyes having an absorption maximum between 420 to 460  $\mu$ , magenta dye-forming couplers which react with the oxidation product of a color developing agent to form magenta dyes having an absorption maximum between 520 to 570  $\mu$ , and cyan dye-forming couplers which react with the oxidation product of a color developing agent to form cyan dyes having an absorption maximum between 630 to 710  $\mu$ . Suitable examples of such couplers are well known in the art, for example, as disclosed in U.S. Pat. Nos. 1,108,028; 2,186,849; 2,206,142; 2,343,702; 2,367,531; 2,369,489; 2,423,730; 2,436,130; 2,474,293; 2,600,788; 2,689,793; 2,728,658; 2,742,832; 2,808,329; 2,998,314; 3,046,129; 3,062,653; 3,265,506; 3,311,476; 3,408,194; 3,419,390; 3,419,391; 3,458,315; 3,476,563; 3,516,831, etc.

These couplers are introduced into the hydrophilic colloid of photographic material using well-known techniques. For example, the couplers can be dissolved in a high boiling organic solvent such as dibutyl phthalate or tricresyl phosphate as described in U.S. Pat. No. 2,322,027, if necessary, in a mixture of the solvent with

a low boiling organic solvent, and the resulting solution is dispersed in the hydrophilic colloid. If the couplers have an acid group such as a carboxylic acid or sulfonic acid group, they can be introduced into the hydrophilic colloid as an aqueous alkaline solution.

To the color photographic light-sensitive material of the invention, there can be also used the "infra-red couplers" described in U.S. Pat. Nos. 2,530,349 and 2,545,687. The "infrared couplers" are couplers capable of forming dyes having a longer wave length than 725  $\mu$  by a coupling reaction with the oxidation product of a color developing agent. By utilizing the optical density of these dyes, the optical density of the silver images in sound track areas can be decreased. That is, the amount of silver coated can be further reduced.

The color photographic light-sensitive materials of the invention is imagewise and sound-imagewise exposed in a conventional manner, and then is processed using conventional color developing steps, which are basically color development, bleach and fixing steps, and if necessary, include a washing step therebetween. After the fixing step, the photographic material is washed and dried, but it is preferred that it be treated with a stabilizing bath before the drying step.

A useful color developer is an aqueous alkaline solution containing a color developing agent. Examples of color developing agents include the well-known primary aromatic amine dye-forming developing agents, for example, the phenylenediamines (e.g., N,N-diethyl-p-phenylenediamine, N-ethyl-N-hydroxyethyl-p-phenylenediamine, N-ethyl-N-hydroxyethyl-2-methyl-p-phenylenediamine, N-ethyl- $\beta$ -N-methanesulfonamidoethyl-3-methyl-4-aminoaniline, N,N-diethyl-2-methyl-p-phenylenediamine, and the sulfates thereof, the hydrochlorides thereof and the sulfites thereof). The color developer can further contain conventional additives such as alkali metal sulfites, carbonates, bisulfites, bromides, iodides or benzyl alcohol. These developing solutions and their components are well known and are described, for example, in C. E. K. Mees and T. H. James, *The Theory of the Photographic Process*, pages 294 - 295, The Macmillan Co., New York, (1966) and in U.S. Pat. Nos. 2,592,364; 2,193,015, etc.

A bleach solution is one which contains conventional bleaching (oxidizing) agents such as ferricyanide or bichromate, and a fixing solution is one which contains conventional fixing agents such as sodium thiosulfate or potassium thiocyanate. The bleach step and the fixing step can be carried out in one bath in the invention, which is impossible in the conventional method requiring sound development. By using such a bleach-fix bath, the processing steps are even more simplified and the processing time is shortened.

The bleach-fix solution in the invention can contain a silver halide solvent which has been used in conventional bleach-fix solutions, such as a water soluble thiosulfate (sodium thiosulfate, potassium thiosulfate, ammonium thiosulfate, etc.), a water soluble thiocyanide (sodium thiocyanide, potassium thiocyanide, ammonium thiocyanide, etc.), a water soluble organic diol fixing agent having an oxygen atom or a sulfur atom (3-thia-1,5-pentanediol, 3,6-dithia-1,8-octanediol, 9-oxa-3,6,12,15-tetrathia-1,17-heptadecanediol, etc.), a water soluble sulfur-containing organic dibasic acid and a water soluble salt (ethylene bisthioglycolic acid, the sodium salt thereof, etc.).

The bleach-fix solution in the invention can contain an oxidizing agent for silver which has been used in conventional bleach-fix solutions, such as a water soluble ferricyanide (e.g., sodium ferricyanide, potassium ferricyanide, ammonium ferricyanide, etc.), a water soluble quinone (e.g., quinone, chloroquinone, methyl-quinone, etc.), a water soluble ferric salt (e.g., ferric chloride, ferric sulfate, ferric thiocyanide, ferric oxalate, etc.), a water soluble cupric salt (e.g., cupric chloride, cupric nitrate, etc.), a water soluble cobaltic salt (e.g., cobaltic chloride, ammonium cobaltic nitrate, etc.). As the oxidizing agent, a polyvalent cation of a water soluble organic acid and an alkali metal complex thereof are preferably used. The organic acid includes compounds represented by the general formulae,



hydroxylamine salt, o-aminophenol, ascorbic acid, semicarbazide, hydrazine, etc.

These bleaching solutions, bleach-fix solutions and the components contained therein are well known to one skilled in the art as disclosed in, for example, *The Journal of the Society of Motion Picture and Television Engineers*, 61, pp. 665-701, and U.S. Pat. Nos. 3,189,452 and 3,582,322.

An example of bleach-fix bath which can be used in the invention is shown by the following formulation,

|                                  |                    |
|----------------------------------|--------------------|
| Bleaching Agent                  | amount shown below |
| Sodium Carbonate (monohydrate)   | 5 g                |
| Boric Acid                       | 5 g                |
| Sodium Sulfite                   | 5 g                |
| Fixing Agent                     | amount shown below |
| Water to make one liter (pH 6.0) |                    |

The bleaching agent and the fixing agent are shown below.

| Bleach-fix Bath | Bleaching Agent                                                                          | Fixing Agent                                                |
|-----------------|------------------------------------------------------------------------------------------|-------------------------------------------------------------|
| a)              | Ferric Sulfate 0.05 mol<br>Disodium Ethylenediamine<br>Tetraacetic Acid 0.1 mol          | Sodium Thiosulfate 0.6 mol                                  |
| b)              | Sodium Ethylenediamine<br>Tetraacetic Acid-Iron(III)<br>Complex Salt 0.1 mol             | "                                                           |
| c)              | Nitrilotriacetic Acid-<br>Iron(III) Complex Salt<br>0.1 mol                              | "                                                           |
| d)              | N-Hydroxyethyl-ethylene-<br>diamine Triacetic Acid-<br>Iron(III) Complex Salt<br>0.1 mol | "                                                           |
| e)              | Sodium Ethylenediamine<br>Tetraacetic Acid-Iron(III)<br>Complex Salt 0.1 mol             | Potassium Thiocyanate 0.6 mol                               |
| f)              | Sodium Ethylenediamine<br>Tetraacetic Acid-Iron(III)<br>Complex Salt 0.1 mol             | Potassium Thiocyanate 0.5 mol<br>Sodium Thiosulfate 0.5 mol |
| g)              | Sodium Ethylenediamine<br>Tetraacetic Acid-Iron(III)<br>Complex Salt 0.1 mol             | Thiourea 0.066 mol<br>Sodium Thiosulfate 0.6 mol            |



wherein X is a hydrocarbon group, a oxygen atom, a sulfur atom or a NR<sub>6</sub> group, R<sub>1</sub>, R<sub>2</sub>, R<sub>3</sub>, R<sub>4</sub> and R<sub>5</sub> each is an unsubstituted or a substituted hydrocarbon group, and R<sub>6</sub> is a hydrogen atom or an unsubstituted or substituted hydrocarbon group.

Examples of these organic acids are malonic acid, tartaric acid, ethyl malonate, malic acid, fumaric acid, diglycolic acid, thioglycolic acid, ethylenedipropionic acid, nitrilotriacetic acid, ethylenediamine tetraacetic acid, aminotriacetic acid, ethylenedithioglycolic acid, dithioglycolic acid, etc.

Examples of polyvalent cations include ferric ions, cobaltic ions, and cupric ions. A complex salt of sodium ethylenediamine tetraacetate with iron is quite useful as the bleaching agent.

The bleach-fix solution of the invention can advantageously contain additives used in conventional bleach-fix solutions, such as sodium sulfite, potassium bromide, potassium iodide, sodium iodide, a polyalkylene oxide, 2-mercaptoimidazole, 3-mercapto-1,2,4-triazole, dithioglycol, thiourea, ethylene thiourea, a

According to the present invention, the color photographic light-sensitive material is exposed and color developed with a color developer, whereby silver images necessary for sound images are formed together with the yellow, magenta and cyan dye images for the color images. Although silver images are formed, in this case, in the color image portions, they are easily removed by the above-described bleach or bleach-fix bath. On the other hand, the silver images formed in the emulsion layers containing the bleach inhibitor are not bleached by the bleach or bleach-fix bath and therefore remain in the layer. Accordingly, according to the invention, sound images (silver images) can be produced using only conventional color development, and the processing steps can be greatly simplified because it is unnecessary to carry out sound development for forming silver images. Namely, silver sound development is not necessary using the light-sensitive material of the invention.

Further, according to the invention, sound track areas of silver images are provided. Therefore, there is the advantage that the decrease of optical density caused by light, heat or humidity is not generated which often results in the sound track areas composed of an organic dye having an absorption in the infra-red region.

In some cases, since a yellow filter layer containing a yellow colloidal silver or an antihalation layer containing a black colloidal silver is provided on the photographic light-sensitive material, which colloidal silver is rehalogenated in the bleaching step and developed in sound development, the photographic material can not be sound developed. On the contrary, according to the invention, since sound development is unnecessary, colloidal silver can be used for the photographic material as the yellow filter layer or antihalation layer.

The invention will be explained in greater detail by reference to the following examples. Unless otherwise indicated, all parts, percents, ratios and the like are by weight.

#### EXAMPLE 1

On opposite surfaces of a cellulose acetate film base, an antihalation layer containing carbon black and a subbing layer were coated. On the subbing layer, a coating composition containing 100 g of a silver iodo-bromide emulsion (silver content 0.05 mol, iodide content 1.2 mol%) and 7.5 g of  $\alpha$ -(2-methylbenzoyl)-3- $\alpha$ -(2,4-di-tert-amylphenoxy)acetoamide-acetoanilide as a yellow coupler which is dispersed in gelatin together with ethyl acetate and dibutyl phthalate was coated to provide a blue-sensitive emulsion layer. On the emulsion layer, a gelatin intermediate layer was coated and then a coating composition containing 100 g of a spectrally sensitized silver chlorobromide emulsion (silver content 0.06 mol, bromide content 30 mol%) and 11.7 g of 1-hydroxy-4-chloro-N-hexadecyl-N-(2-cyanoethyl)-2-naphthamide as a cyan coupler dispersed in gelatin together with ethyl acetate and dibutyl phthalate was coated to provide a redsensitive emulsion layer. The emulsion layer was spectrally sensitized with 0.0015 g of the following spectral sensitizer so as to have a sensitization maximum at about 685  $\mu$ .



On the red-sensitive emulsion layer, a gelatin intermediate layer was coated and then a coating composition containing 100 g of a silver chlorobromide emulsion (silver content 0.06 mol, bromide content 35 mol%) and 2.1 g of 1-(2,6-dichloro-4-methylphenyl)-3-[3- $\alpha$ -2,4-di-tert-amylphenoxy]butylamide-benzamide]-5-pyrazolone and 4.9 g of 1-(2,4,6-trichlorophenyl)-3-[3- $\alpha$ -(2,4-di-tert-amylphenoxy)butylamide-benzamide]-5-pyrazolone as magenta couplers which were dispersed in gelatin together with ethyl acetate and tricresyl phosphate was coated to provide a green-sensitive emulsion layer. The emulsion layer was spectrally sensitized with 0.02 g of the following spectral sensitizer so as to have a sensitization maximum at about 555  $\mu$ .



Then, a coating composition composed of liquid paraffin dispersed in an aqueous gelatin solution was coated on the emulsion layer to provide a protective layer. Thus, a color print film as Sample (I) was obtained.

A color print film as Sample (II) was prepared by coating a composition as a sound track area-forming layer containing 100 g of a silver chlorobromide emulsion (silver content 0.06 mol, bromide content 35 mol%), 0.4 g of Bleach Inhibitor (2), 0.1 g of 4-hydroxy-6-methyl-1,3,3a,7-tetraazaindene and the same spectral sensitizer as used for the green-sensitive layer of Sample (I) between the green-sensitive layer and the protective layer as in Sample (I).

A color print film as Sample (III) was prepared in the same manner as in Sample (II) except that Bleach Inhibitor (2) was not added to the sound track area-forming layer. The coating amount of silver in Samples (II) and (III) each was 1.5g/m<sup>2</sup>.

Samples (I), (II) and (III) each was exposed to a tungsten lamp through an ultra violet absorbing filter transmitting light of a wave length longer than about 400  $\mu$ , a yellow filter transmitting a light of a wave length longer than about 500  $\mu$  and a silver wedge. The filters used in the exposure have been used in the step wedge exposure of usual color print film. Samples (I), (II) and (III) were processed using the following steps A, B and C. The optical densities thus obtained were measured by using a Status S-58 filter using a Macbes TD-206A type densitometer, and are shown in Table 1.

| Processing Step   | Temperature | Time           |
|-------------------|-------------|----------------|
| Pre-bath          | 27°C        | 10 seconds     |
| Washing           | "           | 15 sec.        |
| Color Development | "           | 5 min. 20 sec. |
| Washing           | "           | 15 sec.        |
| First Fixing      | "           | 1 min.         |
| Washing           | 27°C        | 40 sec.        |
| Bleach            | "           | 3 min.         |
| Washing           | "           | 1 min.         |
| Sound Development | 20°C        | 15 sec.        |
| Washing           | 27°C        | 15 sec.        |
| Second Fixing     | "           | 2 min.         |
| Washing           | "           | 5 min.         |
| Stabilizing       | "           | 10 sec.        |

Each processing composition was as follows.

| Pre-bath Solution              |        |
|--------------------------------|--------|
| Water                          | 800 ml |
| Sodium Carbonate (monohydrate) | 10.0 g |
| Sodium Sulfate (anhydrous)     | 50.0 g |
| Water to make one liter        |        |
| Color Developer                |        |
| Water                          | 800 ml |
| Sodium Hexametaphosphate       | 2.0 g  |
| Sodium Sulfite (anhydrous)     | 4.0 g  |
| 2-Amino-5-diethylaminotoluene  | 3.0 g  |
| Hydrochloride                  |        |
| Sodium Carbonate (monohydrate) | 25.0 g |
| Potassium Bromide              | 2.0 g  |

15  
-continued

|                                         |        |
|-----------------------------------------|--------|
| Water to make one liter                 |        |
| <u>First and Second Fixing Solution</u> |        |
| Water                                   | 600 ml |
| Sodium Thiosulfate (pentahydrate)       | 240 g  |
| Sodium Sulfite (anhydrous)              | 15.0 g |
| Glacial Acetic Acid                     | 12.0 g |
| Boric Acid                              | 6.0 g  |
| Potassium Alum                          | 15.0 g |
| Water to make one liter                 |        |
| <u>Bleaching Solution</u>               |        |
| Water                                   | 800 ml |
| Potassium Bromide                       | 20.0 g |
| Potassium Bichromate                    | 5.0 g  |
| Potassium Alum                          | 40.0 g |
| Sodium Acetate (trihydrate)             | 3.0 g  |
| Glacial Acetic Acid                     | 10.1 g |
| Water to make one liter                 |        |
| <u>Sound Developer Solution</u>         |        |
| (Solution A)                            |        |
| Water                                   | 600 ml |
| Sodium Sulfite (anhydrous)              | 40.0 g |
| N-Methyl-p-aminophenol Sulfate          | 40.0 g |

16  
-continued

| Processing C                                                                                        | Processing Step                     | Temperature | Time   |
|-----------------------------------------------------------------------------------------------------|-------------------------------------|-------------|--------|
|                                                                                                     |                                     |             |        |
| 5                                                                                                   | Stabilizing Bath                    | "           | 10 sec |
| Each processing solution was same as in Processing A except for the bleaching solution shown below. |                                     |             |        |
| 10                                                                                                  |                                     |             |        |
| 15                                                                                                  |                                     |             |        |
|                                                                                                     | Ethylenediamine Tetrasodium         | 100 g       |        |
|                                                                                                     | Tetraacetate-Iron(III) Complex Salt |             |        |
|                                                                                                     | Tetrasodium Ethylenediamine         | 18 g        |        |
|                                                                                                     | Tetraacetate                        |             |        |
|                                                                                                     | Ammonium Bromide                    | 160 g       |        |
|                                                                                                     | Aqueous Ammonia Solution            | 5 ml        |        |
|                                                                                                     | Water to make one liter             |             |        |

TABLE 1

| Sample Processing                       | A    | I<br>B | C    | A    | II<br>B | C    | A    | III<br>B | C    |
|-----------------------------------------|------|--------|------|------|---------|------|------|----------|------|
| Optical Density in the Infra Red Region | 1.95 | 0.04   | 0.05 | 2.53 | 1.78    | 2.02 | 2.30 | 0.04     | 0.06 |

|                       |        |
|-----------------------|--------|
| Sodium Hydroxide      | 40.0 g |
| Hydroquinone          | 40.0 g |
| (Solution B)          |        |
| Water                 | 300 ml |
| Tragacanth Gum        | 5.0 g  |
| Denatured Alcohol     | 10 ml  |
| (Solution C)          |        |
| Ethylenediamine (70%) | 20 ml  |

Solution A and Solution B were mixed and, immediately before use, Solution C and water were added to make one liter.

| Stabilizing Bath                   |                 |              |
|------------------------------------|-----------------|--------------|
|                                    | Temperature     | Time         |
| Water                              | 800 ml          |              |
| Formalin (37%)                     | 10 ml           |              |
| Polyethylene Glycol (mol. wt. 400) | 5 ml            |              |
| 40% aqueous Solution               |                 |              |
| Processing B                       | Processing Step |              |
| Pre-bath                           | 27°C            | 10 sec       |
| Washing                            | "               | 15 sec       |
| Color Development                  | "               | 5 min 20 sec |
| Washing                            | "               | 15 sec       |
| First Fixing                       | "               | 1 min        |
| Washing                            | "               | 40 sec       |
| Bleach                             | "               | 3 min        |
| Washing                            | "               | 1 min        |
| Second Fixing                      | "               | 2 min        |
| Washing                            | "               | 5 min        |
| Stabilizing Bath                   | "               | 10 sec       |

Each processing solution was same as used in the Processing A.

| Processing C      |             |              |
|-------------------|-------------|--------------|
| Processing Step   | Temperature | Time         |
| Pre-bath          | 27°C        | 10 sec       |
| Washing           | "           | 15 sec       |
| Color Development | "           | 5 min 20 sec |
| Washing           | "           | 15 sec       |
| First Fixing      | "           | 1 min        |
| Washing           | "           | 40 sec       |
| Bleach            | "           | 3 min        |
| Washing           | "           | 1 min        |
| Second Fixing     | "           | 2 min        |
| Washing           | "           | 5 min        |

From the results shown in Table 1, it is apparent that Samples (I) and (III) must be sound-developed in order to obtain an optical density in the infra-red region, and that Sample (II) need only be color developed in a conventional manner in order to obtain it.

## EXAMPLE 2

35 Sample (IV) was prepared by using 0.1 g of the compound disclosed in U.S. Pat. No. 3,715,208 and represented by the formula,



45 in replace of the Bleach Inhibitor (2) in a sample prepared in the same manner as Sample (II) of Example 1.

The Samples (IV) and (I) to (III) of Example 1 were exposed in the same manner as described in Example 1, and then processed using the following processings D 50 and E. The optical densities thereof in the infra-red region were measured in the same manner as described in Example 1 and are shown in Table 2.

| Processing                  | Temperature                | Processing D |              | Processing E |      |
|-----------------------------|----------------------------|--------------|--------------|--------------|------|
|                             |                            | Step         | Time         | Step         | Time |
| Pre-bath                    | 38°C                       | 10 sec       | 10 sec       | 27°C         |      |
| Washing                     | "                          | 10 sec       | 15 sec       |              |      |
| Color-development           | "                          | 1 min 30 sec | 5 min 20 sec |              |      |
| Stop-fixing                 | "                          | 40 sec       | 2 min        |              |      |
| Washing                     | "                          | 1 min        | 2 min        |              |      |
| Bleach-fixing               | "                          | 1 min 20 sec | 4 min        |              |      |
| Washing                     | "                          | 1 min 40 sec | 2 min        |              |      |
| Stabilizing                 | "                          | 10 sec       | 10 sec       |              |      |
| <u>Stop-fixing Solution</u> |                            |              |              |              |      |
| 60                          | Sodium Thiosulfate         | 240 g        |              |              |      |
|                             | Sodium Sulfite (anhydrous) | 15 g         |              |              |      |
|                             | 28% Acetic Acid            | 48 ml        |              |              |      |
|                             | Boric Acid                 | 7.5 g        |              |              |      |
|                             | Potassium Alum             | 15 g         |              |              |      |
|                             | Water to make one liter    |              |              |              |      |

17  
-continued

| Bleach-fixing Solution                        |         |
|-----------------------------------------------|---------|
| Ethylenediamine Sodium Tetraacetate-Iron(III) | 34.0 g  |
| Complex Salt                                  |         |
| Sodium Carbonate (monohydrate)                | 11.0 g  |
| Boric Acid                                    | 45.0 g  |
| Sodium Thiosulfate                            | 140.0 g |
| Water to make one liter                       |         |

The processing solutions other than the stop-fixing solution and the bleach-fixing solution were the same as those used in Processing A.

TABLE 2

| Processing Sample                       | I    | E    | D    | II   | III  | E | IV |
|-----------------------------------------|------|------|------|------|------|---|----|
| Optical Density in the Infra Red Region | 0.06 | 2.05 | 2.02 | 0.07 | 0.90 |   |    |

From the results contained in Table 2, it is apparent that Sample (II) of the invention provided a higher optical density in the infra-red region by the bleach-fixing bath without sound development, while Sample (I) which is a conventional light-sensitive material and Sample (III) which has a sound track area-forming layer but does not contain the bleach inhibitor do not give a practical density in the infra-red region. When the light-sensitive material of the invention is processed at a high temperature as in Processing D gave similar better results, but Sample (IV) having sound track area-forming layer containing the mercapto compound similarly processed did not to provide sufficient optical density. When Sample (II) is processed by Processing B and C, similar better color images and sound images are obtained.

## EXAMPLE 3

Sample (V) was prepared using 0.15 g of Bleach Inhibitor (1) instead of Bleach Inhibitor (2) using the same procedures as in Sample (II) of Example 1, and Sample (VI) was prepared using 0.20 g of Bleach Inhibitor (4) instead of Bleach Inhibitor (2) as in Sample (II) of Example 1. Samples (V) and (VI) were exposed, and processed in the same manner as in Examples 1 and 2. The thus obtained optical density in the infra-red region was measured and is shown in Table 3.

TABLE 3

| Sample Processing                       | V<br>D | VI<br>D |
|-----------------------------------------|--------|---------|
| Optical Density in the Infra Red Region | 2.10   | 1.84    |

Using Samples (V) and (VI) which are light-sensitive materials of the invention, a higher optical density in the infra red region is obtained.

While the invention has been described in detail and with reference to specific embodiments thereof, it will be apparent to one skilled in the art that various changes and modifications can be made therein without departing from the spirit and scope thereof.

What is claimed is:

1. A color photographic light-sensitive material comprising a support having coated thereon at least one

5 light-sensitive silver halide emulsion layer containing a yellow dye-forming coupler, at least one light-sensitive silver halide emulsion layer containing a magenta dye-forming coupler, at least one light-sensitive silver halide emulsion layer containing a cyan dye-forming coupler, and at least one light-sensitive silver halide emulsion layer containing a compound represented by the following formula,



10 20 wherein R is an alkyl group having at least 12 carbon atoms.

25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 95

19

inhibitor is adjacent said intermediate layer.

9. A process for forming color dye images and silver images which comprises exposing the color photographic light-sensitive material as claimed in claim 2, developing, stopping, first fixing, bleaching and then 5 second fixing said material.

10. The process as claimed in claim 9, wherein said stopping and said first fixing are carried out simultaneously.

11. A process for forming color dye images and silver images which comprises exposing the color photographic light-sensitive material as claimed in claim 2, developing, stopping, bleaching, and fixing said material.

12. A process for forming color dye images and silver images which comprises exposing the color photographic light-sensitive material as claimed in claim 2, developing, bleaching and fixing said material.

13. The color photographic light-sensitive material as claimed in claim 2, wherein said bleach-inhibitor is 20



30

20



or



\* \* \* \* \*

35

40

45

50

55

60

65